

Oct. 16, 1956

J. D. HILL ET AL

2,767,091

METHOD FOR MAKING PAPER

Filed July 25, 1952

2 Sheets-Sheet 1



Inventors:  
Justin D. Hill  
Dean J. Cain  
By: Soans, Glaister & Anderson  
Atty's

Oct. 16, 1956

J. D. HILL ET AL

2,767,091

## METHOD FOR MAKING PAPER

Filed July 25, 1952

2 Sheets-Sheet 2



Inventors:  
Justin D. Hill.  
Dean J. Cain.  
By: Soans, Glaister & Anderson Attns

1

2,767,091

## METHOD FOR MAKING PAPER

Justin D. Hill and Dean J. Cain, Lawrence, Kans., assignors to The Lawrence Paper Company, Lawrence, Kans.

Application July 25, 1952, Serial No. 300,892

4 Claims. (Cl. 92—21)

This invention relates to a novel method for producing a fibrous composition, such as paper, which contains a thermoplastic or waterproofing material, such as bitumen or other heat fusible substances.

The addition of a heat fusible substance, such as bitumen or asphalt, during the paper making process has been heretofore employed in many different ways with varying degrees of success. Indeed, the multiplicity of methods proposed is, of itself, indicative of the many problems existing in the handling of a heat fusible substance in the conventional paper making machinery and of the dissatisfaction with the results of the previous approaches to these problems.

In order to produce a sheet of paper of considerable stiffness and strength with sufficient moisture resisting qualities, it is generally accepted that a relatively large amount of bitumen, or other heat fusible, water-repellant substance, must be added to the ordinary paper stock. The presence of the bitumen in the stock offers a serious problem in being able to adequately control the bitumen so that it does not adhere to the paper machine and thereby interfere with the normal operation of the machine.

Moreover, in the forming of a multi-ply paper board, having at least one inner sheet containing a heat fusible substance, such as bitumen, there has heretofore been considerable difficulty in making a strong, moisture-resistant board without having the bitumen penetrate the outer sheets or liners. The penetration of the liners by the bitumen not only mars the appearance of the finished product, but also presents other deficiencies which detract from the usefulness of the product. The presence of an appreciable amount of bitumen, or other heat fusible substance, on the outer surface of the liners not only permeates the surrounding atmosphere with the odor of the substance but also presents the danger of contaminating food materials and the like which might be contacted by the liners. Furthermore, the striking through of the bitumen, with respect to the liners, naturally results in a decrease in the amount of bitumen bonded between the liners and, therefore, reduces the strength, stiffness, and moisture-resistant properties of the paper board.

Accordingly, it is the principal object of the present invention to provide an improved method for the handling of a thermoplastic, water-proofing material during the making of paper, which will eliminate or minimize the difficulties discussed above, and thereby produce a paper board of improved strength, regulated stiffness, and moisture-proof qualities.

Another object of this invention is to provide a method for uniformly dispersing comminuted particles of a thermoplastic, water-proofing material, throughout a mass of fibrous pulp, and maintaining the uniformity of the mixture during the entire paper making process with a minimum of particle loss in the process.

As a further object of the present invention is to provide novel and improved apparatus for the handling of

2

a thermoplastic, water-proofing material in the manufacture of paper.

These and other objects and advantages of the invention will be made more apparent by reference to the following description and the accompanying drawing, wherein:

Fig. 1 is a diagrammatic showing of apparatus which may be used in making paper in accordance with the present invention.

Fig. 2 is an enlarged sectional view of a portion of the apparatus in Fig. 1.

Fig. 3 is a fragmentary perspective view of a four-ply paperboard made in accordance with the present invention.

According to the invention, a thermoplastic material, such as a hard, dry and friable bitumen, is finely divided and added to the fibrous pulp as the latter is being circulated in a water solution in the beater. The fine particles of the bitumen remain in suspension in the beater and are mixed uniformly throughout the fibrous pulp. The mixture in the beater is then further refined in a Jordan, or similar machine, from which it is fed to a paper making machine of the type having a foraminous, web-forming surface.

The foraminous surface of the paper machine has a mesh which is finer than that normally used in conventional paper making practices to avoid loss of the very fine particles of bitumen. Also, the water used at the wet end of the paper making machine is kept cooled to a temperature below 70° F., contrary to the usual practice, to avoid adherence of the bituminous particles to the machine. The remainder of the treatment of the bitumen and pulp mixture generally follows conventional paper making practices.

Referring to Fig. 1, there is illustrated one embodiment of the invention, wherein the apparatus is indicated diagrammatically, involving the production of a multiply paper board. Whereas the invention will be described with respect to a process involving the use of a bitumen and in connection with cylinder machines, it will be readily apparent as the disclosure progresses that certain of the novel principles set forth herein may be equally applicable to other paper making processes and other web-forming equipment and other thermoplastic materials.

In the making of a four-ply paper board, there is provided a breaker-beater 10 for treatment of the waste-paper, or other stock, to be used in producing a fibrous pulp for the main beater 12 in which the bitumen and pulp are to be mixed prior to forming the paper board. Any suitable means, such as a conduit 14 and a pump 16, may be provided for transferring the pulp from the breaker-beater to the main beater 12.

The main beater 12 is generally of conventional construction, including a beater roll 18, with a slight adaptation to accommodate structure for introducing the bitumen into the beater. Preferably at one end of the beater 12, there is provided a cover 20 which includes a pair of adjacent openings 19 and 21 for the introduction of bitumen into the beater and for the escape of pressure air from the covered portion of the beater, respectively.

For handling the bitumen prior to its addition to the pulp in the main beater 12, there is provided a storage bin 22 having means associated therewith, such as a screw type conveyor 24, for conveying the bitumen to a pulverizing mechanism generally designated by the number 26.

The pulverizing mechanism 26 (Fig. 2) comprises a pair of conventional grinders or hammer mills 28 and 30, respectively, which have been arranged in superposed relation above the cover portion 20 of the main beater 12. More particularly, the upper grinder 28 includes a

cylindrical housing 29 having a top cover 31, and suitable inwardly extending horizontal flange members 33 for supporting the grinder. Suitable bearing means (not shown) are provided in the housing 29 for supporting the center shaft 35 to which is attached a series of radially spaced hammers 36 which grind the material against a breaker bar 37 disposed in the path of movement of the hammers.

The upper portion of the chamber for the grinder 28 also includes a top and side wall forming portion 39 which supports an adjustable gate as well as supporting the lower end of a pipe 38 which extends upwardly through the top cover 31. The pipe 38 affords means for the introduction of a cooling medium, such as compressed air, into the grinders and includes at its outer end a removable cover 40. The adjustable gate 41 is arranged to control the flow of material into the upper grinder chamber.

The lower portion of the grinder 28 comprises a foraminous metal plate or screen 32 which serves as a grading medium for the pulverized material. Metal plates having holes approximately  $\frac{1}{64}$ " in diameter bored therein, in as closely spaced relation as possible, have been used for this screen, but it is to be understood that a standard metal screen of approximately 30 to 40 mesh may also be used.

The lower grinder 30 also includes a cylindrical housing 41 which is disposed in vertical alignment with the housing 29 of the upper grinder and is separated therefrom by a short cylindrical section 43 suitably secured between the two housings 29 and 39. The lower grinder is generally similar to the upper grinder 28, having a center shaft 35', a series of hammers 36' and a breaker bar 37', and is suitably supported in its housing by a pair of plate members 45 which are secured to an upper portion of the housing 41. The grinder 30 also includes a foraminous metal plate 34 at its lower portion which is similar to plate 32. A suitable source of power, such as an electric motor (not shown), is drivingly connected to the center shafts 35 and 35' of the grinders.

Thus it is seen that the bitumen enters the upper grinder chamber, where it is pulverized, and passes downwardly through the screen 32 to the lower grinder 30 where it is further ground. Finally the pulverized particles of bitumen pass through the screen 34 and opening 19 into the main beater 12 where the fibrous pulp is being mixed.

As the finely divided particles fall from the grinders into the beater 12, there is a considerable amount of dust formed in the surrounding air which must be controlled in order to avoid loss of the asphalt and, also, to prevent injury to persons working in the area. The purpose of the cover 20 and the opening 21, which is disposed in close relation to the opening 19 through which the bitumen particles fall, is to assist in controlling this dust.

A vertically extending stack or pipe 44 is positioned over the opening 21 in the cover 20 in communication with the atmosphere, and includes a plurality of shower heads 47 through which water is directed downwardly to settle the dust tending to rise from the beater during the fall of the bitumen particles. It has been found that hot water is most effective in this dust settling operation and, consequently, water having a temperature below the softening point of the bitumen may be satisfactorily used. It should also be noted that the operation of the shower heads 47 is designed to avoid interference with the effectiveness of the pipe 44 as a relief for the air pressure created in the covered portion of the beater during the operation of the grinders and the fall of the bitumen.

After the fibrous pulp and the particles of bitumen have been thoroughly mixed in the main beater 12, the mixture is pumped or otherwise conveyed through a conduit 46 to a Jordan 48, or a similar machine, for further mixing and refining. From the Jordan the pulp mixture is conveyed to the paper making machine in any suitable

way. As shown, the mixture is first pumped to a stock chest 50 and then flows, by gravity or otherwise, to the web-forming equipment which in the present instance comprises two cylinders 52 and 54, respectively, which are used in forming the inner layers of the four-ply board. The flow to the vats of the cylinders 52 and 54 may be controlled by any of the well known means, such as a gate valve controlled by a "spoon" (not shown) in the conduit between the stock chest and the vats.

A separate beater 56 supplies pulp to a second stock chest 58 in the conventional manner to feed the vats for the outer cylinders 60 and 62 which form the non-bituminous outer sheets or liners.

The cylinders 52 and 54, respectively, which form a web from the bitumen-pulp mixture, are conventional except as to the size of the openings in the foraminous cylindrical surface thereof. In lieu of the conventional 50 mesh screen, or larger, on the surface of these cylinders, there is provided a screen of finer mesh in order to avoid loss of the finely divided asphalt particles in the white water. With the described apparatus it has been found desirable to use either a 70 or 80 mesh screen.

Although asphalt does not usually become sticky at temperatures lower than about 125° F. it has been discovered that for some reason not yet known it is very helpful in the prevention of adherence of the bitumen particles to the cylinders and other parts of the machinery to maintain the water in the cylinder at a temperature below 70° F., preferably around 50° F. Then too, it is desirable for most efficient operation in the process to use fresh water in the cylinder vats and new felts at the "wet end" of the paper making machine at the beginning of each "run" of paper stock.

The paper making operation following the formation of the webs on the cylinders involves standard practices with the usual presses and dryers. The temperature of the drying rolls varies from about 220° at the wet end to about 316° at the dry end, and the speed of the paper in this process is related to the temperature and number of drying rolls.

It will be apparent from the foregoing, that the process and apparatus involved is not limited to the making of multi-ply paper. In fact, the procedure has been successfully followed in the making of liners for corrugated boxes, wherein added strength, stiffness and moisture-resistant qualities are important. The above described features which afford advantages in the process, prior to and including the forming of the web on the cylinder, are obviously equally effective without the addition of other sheets or webs to form a multi-ply paper board, as in the described instance.

#### Example

With the foregoing apparatus and method there may be produced a very strong, stiff and moisture-proof paper board by using a hard, dry and friable asphalt having 0 penetration at 77° F. (ASTM D5-25 at 77° F. 100 grams, 5 seconds) and a melting point of between 220° F. and 230° F. (ASTM D3-26). The asphalt is conveyed from the bin 10 to the pulverizing mechanism 26 at a uniform rate of delivery commensurate with the capacity of the grinders which operate at a full load speed of 2400 R. P. M., with screens 32 and 34 having  $\frac{1}{64}$ " diameter openings.

It might be noted at this point that the grinders should not be operated at a speed sufficient to elevate the temperature in the grinders to the melting point of the asphalt. Also, in using the described asphalt and 80 mesh screen on the cylinders 52 and 54, the screens 32 and 34 in the grinders should be of about 30 to 40 mesh, that is having openings of about  $\frac{1}{64}$ " diameter, to obtain the best results. A larger opening in the screens produces particles of sufficient magnitude to strike through the liner of a four-ply paper board under the heat of the dryer rolls. A much smaller opening in the screens re-

quires longer operation of the grinders without any appreciable improvement in the quality of the paper board.

With the grinders operating as described, there is normally no need for cooling the inside of the pulverizing mechanism housing. However, it has been found that under conditions of high temperatures outside of the grinder housing, it may be desirable to cool the inside of the housing by the introduction of compressed air through the pipe 38 at the top of the upper mill 28.

Prior to operation of the conveyor 24 and pulverizing mechanism 26, a waste paper stock is mixed in the breaker-beater 10 and then fed to the main beater 12 until the latter is about half full. This waste paper stock consists mainly of material from old corrugated boxes and waste from new boxes, neither of which contain bitumen or any similar substance.

While the beater roll 18 is down and operating to circulate the waste paper stock, the asphalt is conveyed from the bin 22, through the pulverizing mechanism, and into the beater 12 until the amount of material therein includes 60% stock and 40% asphalt, by dry weight. Specifically, for 1200 lbs. of dry stock there is added 1000 lbs. of asphalt.

During the falling of the asphalt particles from the lower grinder 30 into the main beater 12, a fine spray of hot water is directed down the pipe 44 to prevent loss of asphalt particles through this air vent. The water is preferably kept at a temperature of 190°-200° in order to be most effective as a dust settling means, without causing any objectionable softening of the asphalt particles.

The beater 12 with the asphalt and waste paper stock mixture is then operated for about half an hour in order to disperse the asphalt particles uniformly throughout the stock where they will remain in suspension. Also, once the asphalt particles are in the beater, a small amount of paper-maker's alum may be added to precipitate any unattached asphalt on to the fibers. With the beater containing 2200 lbs. of dry stock and asphalt and 2800 gallons of water, 66 lbs. of alum are added to the mixture in the beater. Thus the added alum constitutes about 3% of the dry weight of the pulp and asphalt. The mixture in the beater 12 is then pumped through the conduit 46 to the Jordan 48 for further mixing and grinding action, and then to the stock chest 50.

Meanwhile, the stock for the liners is prepared in the second beater 56 and delivered to the second stock chest 58. The stock from the two chests is then metered, in the usual way through gate valves controlled by "spoons," through separate conduits to the four cylinder vats. The vats for the cylinders 52 and 54 receive stock from the chest 50 containing the asphalt mixture, and the vats for the cylinders 60 and 62 receive stock from the chest 58 containing the liner stock.

As noted previously, the foraminous surface of the two cylinders 52 and 54, which form sheets 64 and 66, respectively, from the asphalt-containing stock, comprised an 80 mesh screen, as opposed to the ordinary 30-50 mesh screen commonly used on the cylinders in paper machines. The provision of a finer mesh screen is important in keeping the finely divided particles of asphalt from filtering through the cylinder and escaping in the wash water in the cylinder, which action would disturb the uniformity of the mixture as well as diminish the amount of bitumen in the paper formed.

The sheets or webs formed on the cylinders are picked up on the wet felts from which they travel through the usual rolls to the press rolls and dryers. The sheets from the four cylinders are formed, in the course of their travel, into a single sheet 68 of four-ply paper board with the uniformly dispersed bitumen in the inner two sheets 64 and 66 being fused by the heat of the dryer rolls to unite the four sheets which are further bonded together by the compressing action of the calender stacks.

The result of the foregoing process is an improved

multi-ply paper board having added strength and improved moisture-resistant properties over previously known similar products. It is believed that the ability to uniformly disperse very fine particles of asphalt throughout the fibrous pulp and maintain these particles in such relation during the entire process is an important factor in achieving the improved result. The uniformity of the asphalt and fiber mixture and the size of the asphalt particles are undoubtedly important in achieving added strength in the paper board without any appreciable "striking through" of the asphalt or interference with the normal operation of the machinery.

Moreover, by controlling the uniformity of the mixture of pulp and asphalt particles, and the relative quantities thereof, throughout the entire paper making process, it is possible to closely regulate the stiffness of the resulting paper board. Particularly in the manufacture of boxes the dry stiffness quality of the paper board is important and, consequently, it is a definite advantage to be able to control the stiffness as is possible in the disclosed process.

It should be understood that, although the invention has been particularly described with respect to its application to a definite proportion of materials and a particular type of thermoplastic binder and paper stock, other types of thermoplastic binders and paper stocks and relative proportions thereof may be effectively used without deviating from the invention. The percentage of binder material is, of course, dependent upon the results desired. Furthermore, where asphalt has been used in the described process it has been found that an asphalt having a melting point as low as 190° F. is satisfactory. Accordingly, it should be noted that the described example is not intended as a limitation on the scope of this invention.

We claim:

- 35 1. A process for producing paper from a mixture which contains bituminous material and paper-making fiber, said process comprising the comminution of dry bituminous material into air-borne discrete particles all capable of passing a screen not coarser than 30 mesh, while maintaining the temperature of the comminuting zone low enough to prevent fusing and coalescing of the individual particles, passing the air-borne particles directly into a beater containing an aqueous paper-making fiber suspension, said particles being in an amount sufficient to impart a substantial waterproofing property to a sheet of paper made from said mixture, mixing the bituminous particles and fiber to achieve a uniform distribution of the bituminous particles throughout the mixture, and forming a sheet from said mixture on a screen while maintaining the temperature of the sheet-forming zone sufficiently low to prevent fusing and coalescing of the bituminous particles, whereby substantially all of the bituminous material introduced into the beater will be retained in the sheet in the form of uniformly dispersed and discrete particles.
- 40 2. A process for making multi-ply paper wherein at least three fibrous webs are formed, respectively, on separate web-forming machines and combined in superposed relation to form a single sheet of paper, at least one inner web being formed from a paper making furnish including bituminous material in an amount sufficient to impart a substantial waterproofing property to the sheet, said process comprising the formation of said inner web by comminuting the dry bituminous material into air-borne discrete particles capable of passing a screen not coarser than 30 mesh while maintaining the temperature of the comminuting zone low enough to prevent fusing and coalescing of the individual particles, passing the air-borne particles directly into a beater containing an aqueous paper-making fiber suspension, mixing the bituminous particles and fiber to achieve a uniform distribution of the bituminous particles through the mixture, forming a web from said mixture on a screen while maintaining the temperature of the sheet-forming zone sufficiently low to prevent fusing and coalescing of the bituminous
- 45
- 50
- 55
- 60
- 65
- 70
- 75

particles, forming at least two additional webs from an aqueous paper-making fiber suspension substantially free of any significant quantity of bituminous material and placing such webs on opposite sides of said inner web, and drying the multi-ply sheet formed from the superposed webs at a temperature high enough to fuse the bituminous particles.

3. A process for producing paper from a mixture which contains bituminous material and paper-making fiber, said process comprising the comminution of dry bituminous material into air-borne discrete particles all capable of passing a screen not coarser than 30 mesh, while maintaining the temperature of the comminuting zone low enough to prevent fusing and coalescing of the individual particles, passing the air-borne particles directly into a beater containing an aqueous paper-making fiber suspension, said particles being in an amount sufficient to impart a substantial waterproofing property to a sheet of paper made from said mixture, mixing the bituminous particles and fiber to achieve a uniform distribution of the bituminous particles throughout the mixture, and forming a sheet from said mixture on a screen having openings not coarser than 70 mesh, while maintaining the temperature of the sheet forming zone at a temperature not greater than 70° F. to prevent fusing and coalescing of the bituminous particles, whereby substantially all of the bituminous material introduced into the beater will be retained in the sheet in the form of uniformly dispersed and discrete particles.

4. A process for producing paper from a mixture which contains a bituminous material and paper-making fiber, said process comprising the comminution of dry bituminous material having a melting point above 190° F. into air-borne discrete particles all capable of passing a screen not coarser than 30 mesh, while maintaining the temperature of the comminuting zone low enough to prevent fusing and coalescing of the individual particles, passing the air-borne particles directly into a beater containing an aqueous paper-making fiber suspension, said bituminous

5 material comprising about 40 percent, by dry weight, of the solid materials in said mixture, mixing the bituminous particles and fiber to achieve a uniform distribution of the bituminous particles throughout the mixture, and forming a sheet from said mixture on a screen while maintaining the temperature of the sheet forming zone at a temperature not greater than 70° F. to prevent fusing and coalescing of the bituminous particles, whereby substantially all of the bituminous material introduced into the beater will be retained in the sheet in the form of uniformly dispersed and discrete particles.

#### References Cited in the file of this patent

##### UNITED STATES PATENTS

|            |                |                |
|------------|----------------|----------------|
| Re. 15,461 | Perry          | Sept. 26, 1922 |
| 253,655    | Allen          | Feb. 14, 1882  |
| 756,214    | Cornell        | Apr. 5, 1904   |
| 785,025    | Sherwood       | Mar. 14, 1905  |
| 1,515,821  | Avery          | Nov. 18, 1924  |
| 1,621,888  | Kirschbraun    | Mar. 22, 1927  |
| 1,694,523  | White          | Dec. 11, 1928  |
| 1,904,087  | Schacht        | Apr. 18, 1933  |
| 2,022,311  | Fisher         | Nov. 26, 1935  |
| 2,162,687  | Fischer        | June 13, 1939  |
| 2,387,429  | Cate           | Oct. 23, 1945  |
| 2,400,544  | Kline          | May 21, 1946   |
| 2,493,507  | Sutherland     | Jan. 30, 1950  |
| 2,534,703  | Fenelon et al. | Dec. 19, 1950  |
| 2,538,926  | Sutherland     | Jan. 23, 1951  |
| 2,602,029  | Bradshaw       | July 1, 1952   |

##### FOREIGN PATENTS

|         |               |              |
|---------|---------------|--------------|
| 116,040 | Great Britain | May 30, 1918 |
|---------|---------------|--------------|

##### OTHER REFERENCES

Pulp and Paper, by Casey, vol. I, pages 435 and 460, published by Interscience Publishers, Inc., New York (1952). (Copy in Div. 67.)